

## UNITED STATES PATENT OFFICE

2,124,628

PROCESS FOR MANUFACTURING  
LUBRICANTS

Franz Rudolf Moser, Amsterdam, Netherlands,  
assignor to Shell Development Company, San  
Francisco, Calif., a corporation of Delaware

No Drawing. Application March 21, 1935, Se-  
rial No. 12,247. In the Netherlands March 26,  
1934

3 Claims. (Cl. 87—9)

The invention relates to a process for manufacturing lubricants, such as mineral lubricating oils.

It is known to add small quantities of high-molecular monocarboxylic acids, such as oleic acid, stearic acid and cerotic acid, to mineral lubricating oils in order to improve the lubricating property.

The process according to the invention consists in adding to the lubricant carboxylic acids containing two or more carboxyl groups. Such carboxylic acids are much more suitable for the object in view and moreover frequently have still other properties which are of importance in applying the lubricants. Thus, for instance, it has been found that in the case of lubricating oils for cylinders of aero-engines the presence of polycarboxylic acids in these oils results in an appreciably reduced attack of the piston and the cylinder wall through rust-formation.

As higher molecular polycarboxylic acids there may be considered both substituted, e. g. containing groups of hydroxyls or esters, and non-substituted saturated or unsaturated acids. It is essential, however, that more than one free carboxyl group is present.

Suitable polycarboxylic acids are for instance those obtained by a condensation reaction of olefines with maleic acid anhydride, which reaction is related to those described by Diehls and Alder, Ann. 460, page 98 (1928) Ber. 62, page 554 (1928) and Ann. 470, page 62, (1929), and of which the following is a typical example:

200 grams of a highly cracked hydrocarbon distillate boiling from 150° to 200° C. obtained by cracking paraffin wax in the vapor phase and having a bromine number of 116 is heated with 140 grams maleic acid anhydride during 14 hours at 150—160° C. and then for 30 hours at 200—230° C., whereafter it is fractionated under a vacuum of 13 mm. mercury. 146 grams of a fraction boiling from 155 to 165° C. are subsequently hydrated by boiling for 2 hours with 500 milliliters of water to produce the free acid. Upon extraction with ether an extract amounting to 155 grams of light yellow acid-reacting viscous oil is obtained.

When adding .25 to .5% of this acid to a mineral lubricating oil, the resulting blended oil is

capable of effectively preventing corrosion of internal combustion engines, whether such engines have been in use or not.

Another suitable acid is agaric or 1-cetyl citric acid (Chem. Abst. 25, page 1213, 1931). 5

Further examples are polycarboxylic acids obtained by polymerization, e. g., by heating and/or boiling, voltolizing, etc., of fatty acids, or acids produced from polymerized fats by hydrolyzing, or saponifying same and liberating the acids 10 from the soap.

The added quantities of polycarboxylic acids are, as a rule, comparatively small, e. g. less than 5%, in many cases even below 1%.

## Example I 15

The addition of 0.5% voltolized oleic acid to a mineral lubricating oil, either compounded or not, is sufficient to obtain the above effect when using the oil as lubricant for cylinders of aero-engines. 20

## Example II

A technical quick-drying oil, upon the soap-solution obtained being saponified and acidified, yields a polycarboxylic acid-containing product 25 which when added in a quantity of 1% to a mineral lubricating oil has the property of preventing rust-formation in aero-engine cylinders.

I claim:

1. A lubricant capable of reducing corrosion in 30 internal combustion engines, consisting essentially of a mineral lubricating oil containing as an active anticorrosion ingredient a small quantity of a polycarboxylic acid obtained by condensation of maleic acid anhydride and olefines. 35

2. A lubricant capable of reducing corrosion in internal combustion engines consisting essentially of a mineral lubricating oil containing as an active anti-corrosion ingredient less than 5% of a polycarboxylic acid obtained by condensation 40 of maleic acid anhydride and an olefine.

3. A lubricant capable of reducing corrosion in internal combustion engines consisting essentially of a mineral lubricating oil containing as an active anti-corrosion ingredient less than 1% 45 of a polycarboxylic acid obtained by condensation of maleic acid anhydride and an olefine.

FRANZ RUDOLF MOSER.